# EUROPEAN PATENT SPECIFICATION

(11) **EP 1 598 455 B1**
(45) Date of publication and mention of the grant of the patent: **03.06.2009**
(21) Application number: 04381014.2
(22) Date of filing: 20.05.2004
(51) Int. Cl.: D01F 9/133, F27B 1/02

(54) **Furnace and procedure for the manufacture of carbon fibres**
Ofen und Verfahren zur Herstellung von Kohlenstofffasern
Four et procédé pour la production de fibres de carbone

(43) Date of publication of application: 23.11.2005
(73) Proprietor: Grupo Antolín Ingeniería, S.A., 09007 Burgos (ES)
(72) Inventor: Merino Sanchez, Cesar, 09230, BUNIEL (BURGOS) (ES); Soto Losada, Pablo, 09006, BURGOS (ES)
(74) Representative: Capitan Garcia, Maria Nuria

(56) References cited:
- EP-A1- 1 277 858
- EP-A1- 1 375 424
- EP-A2- 0 969 127

## Description

### OBJECT OF THE INVENTION

The present invention refers to a furnace for the manufacture of carbon fibres consisting of a set of reaction tubes as well as the auxiliary installation required for its operation. The procedure for obtaining those carbon fibres using said furnace as well as the fibre obtained form part of this invention.

The furnace of the present invention is characterized by a configuration in the manner of a set of reaction tubes vertically placed forming a single block with common heating system.

This layout with common heating system reduces the heat losses increasing the energetic efficiency of the reaction without the modularity and scalability of the furnace being affected.

The independence of each of the reactor tubes allows individual control and feed adjusted to the actual carbon fibres manufacturing conditions as well as the possibility of carrying out cleaning of each of the tubes without production being interrupted in the remainder.

The use of a common collector for fibre collection and residual gas outlet and its configuration allow greater simplicity and simplification of the installation.

Furthermore the installation is configured as a closed and gas-tight circuit avoiding the escape of gases and allowing the reuse of the residual process gas giving as result a process with a notable saving by having avoided part of the supply of reagent gases. It should be emphasized that it is verified in practice that the residual gas is of a quality that is equivalent to that of the gases used as raw material.

The fibre (or nanofibre considering its dimensions) obtained by this procedure is characterised by the structure and properties arising from the process used.

### BACKGROUND OF THE INVENTION

Carbon nanofibres are carbon filaments of submicrometric size with a highly graphitic structure, grown in the vapour phase (usually called s-VGCF "submicron vapour grown carbon fibres") that are located between carbon nanotubes and commercial carbon fibres, even though the limit between carbon nanofibres and multiwall nanotubes is not clearly defined.

Carbon nanofibres have a diameter generally between 30nm and 500nm and a length greater than 1µm.

Scientific literature exists in which both the physical-chemical characteristics of the nanofibre and the process of creation at microscopic level from the carbon source used for obtaining it, are described and modelled.

These models have been created in most of the cases based on laboratory experiments making use of controlled atmospheres combined with observations with electronic microscopes whether scanning or transmission.

Carbon nanofibres are produced by catalysis from the decomposition of hydrocarbons on metallic catalytic particles originating from compounds with metal atoms, forming nanometric fibrilar structures with highly graphtic structures.

Studies exist such as those of Oberlin [Oberlin A. et al., Journal of Crystal Growth 32, 335 (1976)] in which the growth of carbon filaments on metallic catalytic particles is analysed by transmission electronic microscopy.

Based on these studies, Oberlin proposed a growth model based on the diffusion of carbon around the surface of the catalytic particles until the surface of the particles is contaminated by an excess of carbon.

Similarly he explained that deposition due to thermal decomposition of carbon is responsible for the thickening of the filaments, and that said process takes place along with the growth process, and in consequence is very difficult to avoid.

For this reason, once the growth process has ended, for example by contamination of the catalytic particle, the thickening of the filament continues if the conditions of pyrolisis continue to exist.

Afterwards other growth models have been proposed that have been equally examined in view of experimental data and starting from various simplified hypotheses that give rise to results that adjust to a greater or lesser degree with the observations made in laboratory.

The metallic catalytic particles are formed by transition metals with atomic number between
21 and 30 (Sc, Ti, V, Cr, Mn, Fe, Co, Ni, Cu, Zn), between
39 and 48 (Y, Zr, Nb, Mo, Tc, Ru, Rh, Pd, Ag, Cd), or between
73 and 78 (Ta, W, Re, Os, Ir, Pt). It is also possible to use, Sn, Ce, and Sb, those of Fe, Co and Ni being especially indicated.

Different chemical compounds can be in use as a source of metallic catalytic particles for the continuous production of carbon nanofibres, such as inorganic and organic metallic compounds.

A huge jump exists as to means and methods of production from laboratory results to the obtaining of industrial quantities of nanofibre in acceptable conditions from the engineering and economic cost point of view.

At industrial level the ways of preparing the catalytic metallic particles for their introduction into the reaction furnace can be classified into two groups: with substrate and without substrate.

In the first case, when the metallic particles are provided with substrate, fibres are obtained for applications for which it is of interest that they be aligned as is the case of their use in electron emission sources for microelectronic applications.

In the second case, also called floating catalyst, the reaction is carried out in a given volume without the metallic particle being in contact with any surface, having the advantage that later afterwards it is not required to separate the nanofibres produced from the substrate.

It is very improbable that the carbon nanofibres grow directly from the initial carbon source. It is believed that the filaments appear from secondary products created from the thermal decomposition of the initial carbon source.

Some authors mention that for light hydrocarbons lower than C₁₆ any of them can be used, without the quality of the nanofibre obtained depending on the hydrocarbon chosen.

Carbon nanofibres are used to make filled polymers giving rise to materials with improved properties, such as tensile strength, Young's modulus, electrical conductivity and thermal conductivity. Others applications are, for example, their use in tires partially replacing carbon black, or in lithium-ion batteries since the carbon nanofibres are easily intercalated with lithium ions.

After examining the nanofibre growth models it has been commented that deposition due to thermal decomposition of carbon is responsible for the thickening of the filaments produced along with the growth process, and that such thickening continues if the conditions of pyrolisis continue to exist. As a consequence, in an industrial furnace the thickening continues if the nanofibre is kept in the reactor.

The residence time of the fibres in the reactor is very important since the greater the residence time, the greater the diameter of the fibres produced.

The manufacture of this type of nanofibre in industrial processes has been considered by means of techniques such as that described in the Japanese patent JP60027696, where use is made of a number of reaction tubes placed horizontally and in parallel to work in the vapour phase and with the catalyst fixed on a substrate.

In these type of reaction tubes the collection of the fibre is discontinuous since it grows on the substrate where the latter is covered with catalytic particles.

As the patent describes, also in this device resistances positioned in block with thermal insulation are used.

In general, when the floating catalyst technique is used with horizontal furnaces there is the disadvantage that either one works with very high gas flows that are capable of drawning the fibre produced to the outside of the furnace, or the fibres, once created, can remain inside the furnace a fairly long time, with the consequent loss of properties due to the thickening as a consequence of the deposition of pyrolitic carbon on the surface of the fibre.

In the vertical furnace, in contrast, it is possible to have greater control of the residence time of the fibres produced inside the furnace, and thus to avoid the unwanted thickening of the fibres due to pyrolitic deposition of carbon.

The present invention consists of a new design for the furnace that allows continuous production of high quality fibre and with reduced costs, along with the auxiliary installation that supplies it, to be obtained.

### DESCRIPTION OF THE INVENTION

The object of the present invention is a furnace for the manufacture of carbon fibres that has a set of auxiliary elements for its correct supply and evacuation of both the reaction gases and the fibre obtained, as well as allowing the periodic and independent cleaning of each of the tubes that make up the furnaces.

This furnace consists of a set or grouping of tubes, preferably ceramic in order to avoid problems of corrosion due to the reagent gases, placed in a vertical position.

The heating of the tubes to reach the pyrolisis temperature of the hydrocarbon is carried out by means of a block of resistances covered with thermal insulation, that prevents escape of heat to the outside. By being a common block the construction is simple and the insulation more effective, avoiding to the maximum temperature loss, optimizing the use of electric power necessary for heating. This common block of resistances can however be formed as a grouping of the individual resistances of each reactor tube forming a single set, for example because the reactor tubes are fabricated with the resistance incorporated.

The ceramic tubes are completely within the block of resistances. The union of the ceramic tubes to the rest of metallic parts of the installation is carried out using metallic tubes, both in the upper and in the lower part of each ceramic tube. A number of jackets, through which a cooling liquid circulates, surround the metallic tubes, to have low temperature at the points of contact of the ceramic and metallic material, and to prevent rupture of the ceramic material, caused by the different thermal expansion of the materials, as well as the possible burning of the closing and sealing joints between both tubes.

Each of the tubes is feeded, independently from the others, with catalyst, hydrocarbon and a diluting gas such as, for example, hydrogen.

Feed is carried out at a pressure greater than atmospheric before entering the tube, whereas the fibre collector forms part of a recirculation circuit working at a pressure lower than atmospheric pressure.

As well as each tube being independently feeded, it also has independent outlet valves, so that any of the furnaces can remain out of service without affecting the rest of the installation.

One of the reasons for which it is of interest to isolate any tube is that of cleaning.

Although most of the production of fibre takes place in the core of the descending gas flow (without substrate), it is possible that some particle of catalyst may enter in contact with the wall of the furnace tube.

The growth of fibre from these particles deposited on the wall is what gives rise to the existence of an accumulation of fibre on the walls, dirtying and gradually obstructing the tube.

The procedure of cleaning the tube is carried out without stopping the productive process in the furnace, but rather that the tube that requires to be cleaned is isolated closing the lower valves and the hydrocarbon and catalyst feed valves.

Once the inert gas has swept any remains of reaction gases, the feed is replaced with air and therefore with a supply of oxygen.

The presence of oxygen produces the combustion of the carbon that is swept away and eliminated. Once the combustion has been completed, the furnace is again fed with the inert gas, until it eliminates the oxygen.

Nitrogen is a gas that it is possible to consider inert at the working temperatures of the furnaces and it is of low cost, although it is possible also to use noble gases in the case of it being necessary.

After this operation the furnace is ready to continue producing, so that the catalyst, hydrocarbon and diluting gas feed valves are again opened.

The fibre obtained in each of the tubes comes to a single sloping collector that facilitates drawning, both by gravity and by the flow forced by means of a residual gas impeller, to a pressurized collection tank. This single collector results in a simplified installation that avoids a large number of bends and valves that create stagnation and discontinuous flow in the collection of the nanofibre.

Both the valves placed to the outlet of each of the tubes and the oblique collector are elements that form part of this invention.

The residual gas is re-circulating in a circuit part of which is formed by the collector. The residual gas impeller mentioned previously is that entrusted with this recirculation.

The residual gas, adequately treated and pressurized until reaching the feed pressure, is partially re-used, drastically reducing the cost requirements for raw material.

The mass-flow control of each of the reagents, of the dilutent and of the residual gas used in the back-feed is carried out by means of a control system that adjusts the appropriate values for each of the furnaces. Every furnace has its independent feeding and the valves necessary for isolating it or for connecting it with the rest of the installation.

The fibre obtained by this procedure has a very high degree of homogeneity as regards dimensional parameters (diameter and length), as well as mechanical characteristics (modulus of elasticity and tensile strength), and physical (thermal and electrical conductivity) very interesting for its industrial use.

With respect to the procedure used in obtaining the fibre using the furnace, including the individualized cleaning stages of each of the tubes, this gives rise to a viable process by means of the installation described that turns out to be economically productive using commercial sizes of ceramic tubes. The manufacture of tubes with other special sizes implies amortization in the long term and an increase in price of the carbon nanofibre produced.

The use of a furnace that consists of independent reaction tubes facilitates the scaling of a plant in accordance with the production required, needing only the installation of more or less tubes. Because of the setup and advantages stated previously, any size of installation can be made, from one tube up to any number, depending on the need for production required.

### DESCRIPTION OF THE DRAWINGS

This descriptive report is supplemented by a set of drawings, illustrative and never limitative, of the preferred example of the invention.

Figure 1 shows a schematic diagram of an embodiment of the invention consisting of the set of reaction tubes, as well as the auxiliary parts that complete the installation to carry out the obtaining of fibre.

Figure 2 shows a histogram obtained from a statistical reading of the average diameter with a high sampling size for the fibre manufactured by means of the installation that is object of the invention. On this histogram the corresponding fit normal or Gauss probability density function is shown.

### DETAILED EXPOSITION OF A MEANS OF EMBODIMENT

Figure 1 is a schematic diagram of a possible embodiment of the invention that uses a furnace formed by four vertical tubes (1, 2, 3, 4), of the same diameter and length, forming a single block (5) lined with resistances and insulation. The temperature at which the reaction takes place is between 800 and 1500°C, reached by means of the heating of the resistances.

The feeding of the components to the reaction tubes (1, 2, 3, 4) is carried out via their top part and the output of the nanofibres and the residual gas of the reaction via its lower part.

Both zones, input and output of the reaction tubes (1, 2, 3, 4), must be at temperatures lower than those of the reaction, in the case of the input of components to protect the dosing devices, and in case of the output of the product in order that this may be collected, and so that the gases lose part of their chemical activity, it being thus possible to handle them.

For this purpose, in the upper and lower ends of each of the tubes (1, 2, 3, 4) that make up the furnace there is a metallic tube with a refrigerating jacket (30) through which a refrigerated liquid circulates, supplied by means of hydraulic pipes (31). Furthermore, at the points of contact of the ceramic and metallic material a low temperature must exist, and to prevent rupture of the ceramic material being produced, caused by the different dilation of the materials, as well as the possible burning of the closing and sealing joints between both tubes.

In the lower part of the tubes (1, 2, 3, 4) and in each of them, there is a valve (6) that leads to the collector (7) that collects the product of the reaction, carbon nanofibres and the residual gas.

The collector (7) is a collection pipe with an essentially closed ring configuration. In this ring there are two more important parts: in addition to the pipe in the strict sense there is a impeller (8) of gases that provides the thrust necessary for the circulation of the gases and the nanofibre always in the same direction, and a system of nanofibre collection (9) without detaining the gas flow.

The collector part (7) placed under the tubes (1, 2, 3, 4) has a slope that facilitates the conduction of the carbon nanofibres down to the nanofibre collection device (9). In this device the separation of nanofibre and gases takes place, the nanofibre remains stored without blocking the way of the residual reaction gas which continues its way inside the collector ring (7).

From the system of collection (9) only gases circulate until they again encounter the nanofibres and the output gases of the reaction tubes.

Within this closed ring and in the reaction tubes the pressure is constant and less than atmospheric, between -1 and -200 mbar. In the rest of the installation a constant relative overpressure of between 100 mbar and 1 bar exists.

The difference of pressures between the supply zone and that of output in the installation is obtained principally using means (32) of pressure control, this being set within a range.

The components that form part of the chemical reaction are introduced through the upper part of the tubes (1, 2, 3, 4). Said components are:
- A compound with catalytic metallic content, in vapour phase (10), preferably all of them with a transition metal and, especially, iron, cobalt or nickel. For example, ferrocene or iron pentacarbonile,
- a hydrocarbon (11) such as natural gas or other industrial gases,
- a diluting gas (12), for example, hydrogen,
- recirculation gas, introduced through the recirculation pipe (13).

The use of natural gas as a source of carbon obligates the use of ceramic reaction tubes. Natural gas is composed principally of methane, and in small quantities of other components, specifically, some of them are sulphur compounds. These sulphur compounds and the temperature at which the reaction is carried out corrode iron and any metallic alloy. Some ceramic materials are inert for any type of reaction, both reduction and oxidizing, and therefore ideal as material for using in reaction tubes.

All of the components, except the compound source of metallic catalytic particles, with which each of the furnaces is fed, are dosed in their appropriate quantities by means of mass-flow controllers (14, 15, 16, 17), one for each gas and reaction tube. Thus, for four reaction tubes (1, 2, 3, 4) and three process gases, there are 12 mass-flow controllers, such as those represented in the schematic diagram of the figure.

In each reaction tube (1, 2, 3, 4), the components are introduced via the high part of the tubes (1, 2, 3, 4) through pipes (18, 33) in which there are valves (19, 20) whose function will be indicated hereinafter.

During the chemical reaction by which the carbon nanofibres are formed within the reaction tubes some metallic catalytic particles are also deposited on their internal walls from which growth of carbon fibre takes place.

This fibre is maintained bonded to the internal walls of the reaction tubes (1, 2, 3, 4) and attracts others metallic catalytic particles. In this way carbon nanofibres grow continuously from the internal walls of the tubes (1, 2, 3, 4), that could manage to decrease the production in said tubes (1, 2, 3, 4).

For this reason, it is necessary to carry out consistent cleaning by burning the carbon nanofibres achieving their detachment and drawing away for their evacuation.

### Cleaning procedure of a reaction tube

When it is required to carry out the cleaning of a reaction tube, in first place the production of carbon nanofibres is stopped, and for this purpose the supply valves of the reagent components (19) and (20) and the reaction product collection valve (6) in the lower part of the tubes are closed.

After this valve (21), through which an inert gas is introduced to stop the chemical reaction and a valve (26) for the evacuation of the gases are simultaneously opened. Nitrogen, for example, is introduced as an inert gas.

The inert gas is introduced through a pipe (23) that has branchings to each reaction tube, whose passing is controlled by means of the valves (21) already mentioned.

This inert gas draws away gases and nanofibres of the reaction to the lower part of the reaction tubes (1, 2, 3, 4), passing out through the pipe (25) of each reaction tube and passing through the valve (26) to reach the common collection pipe (27) which in turn discharges into a means of collection (28) of nanofibres and gases.

In the common pipe (27) a control system (29) exists that detects when the reagent gases have been expelled, that is, when so-much per cent of gaseous hydrocarbons in this output is below a minimum.

At this moment the inert gas pass valve (21) is closed and the input valve (22) for air that circulates through the pipe (24) is opened. The carbon reacts with the oxygen of the air producing the combustion and release of the nanofibres from the internal wall of the tubes (1, 2, 3, 4), which are drawn away to the means of collection (28) of ashes and gases.

The introduction of air continues until the analyzer (29) stops detecting carbon monoxide and dioxide that are the principal compounds formed by combustion of the nanofibres.

At this moment the air introduction valve (22) is closed and the inert gas introduction valve (21) is again opened. This is done to clean the tube (1, 2, 3, 4) of oxygen and they are kept open until the analyzer (29) does not detect oxygen.

At this moment the inert gas introduction valves (21) and evacuation valves (26) are closed and the fibre production and residual gas output valves (6) and hydrocarbon and diluting gas supply (19) valves and that of catalyst supply (20) are opened to restart the production of carbon nanofibres.

### Procedure for obtaining the fibre in production

The production of fibre by means of the installation described uses as many tubes (1, 2, 3, 4) as are necessary to meet the required production it being possible to scale the furnace as much as needed, in the number of reactor tubes along with the valves associated with feed, evacuation and cleaning.

The layout of the tubes (1, 2, 3, 4) forming a grouping allows that the production of nanofibre and their surface cleaning can be carried out independently, thus using any combination of the tubes (1, 2, 3, 4) with each other. In this way it is possible to have tubes that are being cleaned and tubes that are producing carbon nanofibres at the same time.

It is also possible, given a certain number of available furnaces, to adjust the production levels using only some of them keeping the rest with the valves closed and therefore out of service with neither the efficiency nor the quality of the carbon nanofibre production being reduced.

In this way, the cleaning procedure of a reaction tube can be considered to be a sub-stage of the production procedure for the use of the furnace according to the invention as well as of the rest of the auxiliary elements.

### Fibre obtained

From the production conditions described carbon nanofibres have been manufactured on which various analyses are carried out to determine their quality and their structural characteristics.

By means of their observation by microscope at different scales a very high degree of dimensional homogeneity and the absence of impurities is observed.

From the statistical point of view various dimensional readings have been carried out both of the diameter and of the length of the fibre obtained.

These parameters depend principally on the quality of the reaction conditions, on the activity of the metallic catalytic particle, and on the permanence time of the catalytic particle in the reaction conditions without it becoming contaminated.

Figure 2 corresponds to a histogram corresponding to a sampling size of the diameter of 311 readings sufficient enough to establish an approximation of the probability density function.
This function has been fitted using a normal or Gauss function that is shown superimposed on the histogram.

For the estimation of the average a value of 122.96 nm. has been obtained and for the standard deviation 33.16 nm. all of the samples being within the range [32.25, 228.09]. Standard deviations less than 40nm. are appropriate dispersion values for most of the applications.

Fibre diameters of between 30 and 500 nm. are accepted as valid, the fibre manufactured not being rejected because samples outside of these values are found but rather that they are accepted when the average and the standard deviation indicate that a large percentage of the fibres fabricated are in this interval.

An acceptable production would be to consider that 80 % of the area corresponding to the of normal normal or Gauss probability density function used in the samples fit are within the interval [30,500] in nanometres for a sufficiently representative sample.

Similarly a production in which the average of diameter variable obtained on the Gauss or normal probability density function used in the fit was within the range [80 nm, 180 nm] in these cases being that much better the lesser the degree of dispersion.

In this same example fibres have been obtained whose length is between 20 and 200 micrometers. In this case the length has a very high variance and its validity highly depends on the later application of the fibre.

## Claims

1. Furnace for the manufacture of carbon fibres **characterised by** consisting of a number of vertically positioned ceramic tubes (1, 2, 3, 4), with a common block of resistances covered by an insulating element forming a single block (5), where the upper and lower ends of the tubes (1, 2, 3, 4) are connected to metallic tubes with refrigerating jackets (30); the tubes (1, 2, 3, 4) are fed from above through pipes (18, 33) fitted with pass valves (19, 20); and each of them having in its lower end, after the passing of the fibre through the reaction tube (1, 2, 3, 4), a pass valve (6) connected at an end to each of the metallic tubes corresponding to each tube (1, 2, 3, 4), and at the another end to a single collector (7).

2. Furnace for the manufacture of carbon fibres according to claim 1 **characterised in that** the common block of resistances is constituted as a grouping of individual resistances associated with each reaction tube (1, 2, 3, 4).

3. Furnace for the manufacture of carbon fibres according to claim 1 **characterised in that** it has jackets (30) that surround the upper and lower ends of the reaction tubes (1, 2, 3, 4) through which cooling liquid circulates for the reduction of the temperature in such ends below the temperature of pyrolisis.

4. Furnace for the manufacture of carbon fibres according to claim 1 **characterised in that** the supply of hydrocarbon (11), dilutent (12), recycled gases (13), is carried out by the apportioning of the quantities by means of mass controllers (14, 15, 16, 17).

5. Furnace for the manufacture of carbon fibres according to claim 1 **characterised in that** the collector (7), at least in the fibre and residual gas reception section, has an inclination to facilitate the evacuation of both of these.

6. Furnace for the manufacture of carbon fibres according to claim 1 **characterised in that** the collector (7) is shaped as a closed ring with a gas impeller (8) with capacity to generate gas velocities sufficient to achieve the drawing away of the fibre produced.

7. Furnace for the manufacture of carbon fibres according to claim 6 **characterised in that** the ring collector (7) is interrupted by a fibre collection device (9) that does not block the passing of the recirculating gas.

8. Furnace for the manufacture of carbon fibres according to claim 6 **characterised in that** all of the installation is gas-tight.

9. Furnace for the manufacture of carbon fibres according to claim 1 **characterised in that** there exists a back-feed pipe (13) that leads the gas from the residual gas recirculation collector (7) to the feed.

10. Furnace for the manufacture of carbon fibres according to claim 9 **characterised in that** in the back-feed pipe (13) there exist means of control (32) of the pressure of the recirculating gas, to adjust it, within a range, to the feed pressure.

11. Furnace for the manufacture of carbon fibres according to claim 1 **characterised in that** it has an alternative feed and of evacuation pipes in the lower part of each of the tubes (1, 2, 3, 4) reactors that lead to an ash collection system (28) for the individualized cleaning of each reactor tube (1, 2, 3, 4).

12. Furnace for the manufacture of carbon fibres according to claim 11 **characterised in that** the cleaning alternative feed consists of two pipes, one of air (24) and other of an inert gas (23), each one of them with its valve (22, 21) placed before the input to the reactor tube (1, 2, 3, 4).

13. Furnace for the manufacture of carbon fibres according to claim 12 **characterised in that** the inert gas is nitrogen.

14. Furnace for the manufacture of carbon fibres according to claim 12 **characterised in that** the inert gas is a noble gas.

15. Furnace for the manufacture of carbon fibres according to claim 11 **characterised in that** the means for evacuation in the cleaning operations consist of pipes (25) that converge into a single one and each of them has its valve (26) placed at the output of each reactor tube (1, 2, 3, 4).

16. Furnace for the manufacture of carbon fibres according to claim 11 **characterised in that** the cleaning output (27) has a control system (29) for determining the moment in which the cleaning operation has ended.

17. Procedure for the obtaining of carbon fibre using a furnace according to the previous claims which consists of a continuous process of fibre obtention by pyrolysis of the hydrocarbon and the growth of fibre in the vapour phase from metallic catalytic particles, in all or in part of the reaction tubes (1, 2, 3, 4) with a hydrocarbon feed (11) **characterised in that** it is also feed with a catalyst (10), and a dilutent (12) plus recycled gases (13) in proportions determined by a control system that by means of mass-flow controllers acts independently on each of the reactor tubes (1, 2, 3, 4); being applied a cleaning stage on any of the tubes (1, 2, 3, 4), according to the degree of accumulation of fibre in the interior, without this stage interfering in the production of the remainder of the tubes (1, 2, 3, 4); and, as soon as the cleaning stage has been applied to a given tube, to return this latter to production conditions collection of the fibre being established in a means (9) of collection and storage.

18. Procedure for obtaining carbon fibre according to claim 17 **characterised in that** during the production of carbon fibre reaction tubes (1, 2, 3, 4) exist in production and others simultaneously in cleaning without the global production process being stopped by the cleaning operation.

19. Procedure for the obtaining of carbon fibre according to claim 18 **characterised in that** the cleaning of a reaction tube (1, 2, 3, 4) consists of the following stages
• closing of the feed valves (19, 20) and of the evacuation valve (6) isolating the tube from the rest of the installation.
• opening of the inert gas feed valve (21) for the detention of the reaction of carbon fibre formation, and of the valve (26) of access to the gas and ash evacuation pipe (25),
• maintenance of the inert gas feed until a control system (29) detects the absence of hidrocarbonated compounds,
• closing of the inert gas feed valve (21),
• opening of the air feed valve (22) for combustion of the carbon fibre with oxygen in high temperature conditions,
• continuing of the feed of air until a control system (29) confirms the extinction of the combustion reaction, preferably by detecting the presence of carbon and oxygen compounds,
• as soon as the combustion reaction has finished, the air input valve (22) is closed and the inert gas input valve (21) is opened until the oxygen has been completely eliminated, as detected by the control system (29) due to the absence of carbon and oxygen compounds,
• the inert gas feed valves (21) and the gas and ash evacuation pipe valve (26) are closed,
• the feed valves (19, 20) and gas and fibre output valves (6) are again opened, production being again established in this tube.

## Patentansprüche

1. Ofen zur Herstellung von Kohlenstoff-Fasern, **dadurch gekennzeichnet, dass** dieser aus einer Anzahl vertikal angeordneter Keramikrohre (1, 2, 3, 4) mit einem gemeinsamen durch ein Isolierelement abgedeckten Widerstandsblock in Form eines einzigen Blocks (5) besteht, wobei die oberen und unteren Enden der Rohre (1, 2, 3, 4) mit Metallrohren mit Kühlmänteln (30) verbunden sind, die Rohre (1, 2, 3, 4) von oben über mit Durchlassventilen (19, 20) ausgerüstete Rohrleitungen (18, 33) gespeist werden und jedes dieser Metallrohre an seinem unteren Ende, nach Durchlauf der Fasern durch das Reaktionsrohr (1, 2, 3, 4), ein Durchlassventil (6) aufweist, das an einem Ende mit jedem der Metallrohre entsprechend dem jeweiligen Rohr (1, 2, 3, 4) und am anderen Ende mit einem einzigen Sammler (7) verbunden ist.

2. Ofen zur Herstellung von Kohlenstoff-Fasern nach Anspruch 1, **dadurch gekennzeichnet, dass** der gemeinsame Widerstandsblock aus einer Gruppe von einzelnen, einem jeden Reaktionsrohr (1, 2, 3, 4) zugeordneten Widerständen besteht.

3. Ofen zur Herstellung von Kohlenstoff-Fasern nach Anspruch 1, **dadurch gekennzeichnet, dass** dieser Mäntel (30) umfasst, welche die oberen und unteren Enden der Reaktionsrohre (1, 2, 3, 4) umgeben und durch die eine Kühlflüssigkeit zur Absenkung der Temperatur in diesen Enden unter die Pyrolysetemperatur strömt.

4. Ofen zur Herstellung von Kohlenstoff-Fasern nach Anspruch 1, **dadurch gekennzeichnet, dass** die Zuführung von Kohlenwasserstoff (11), Verdünner (12), rückgeführten Gasen (13) durch Dosierung der Mengen mit Hilfe von Massereglern (14, 15, 16, 17) erfolgt.

5. Ofen zur Herstellung von Kohlenstoff-Fasern nach Anspruch 1, **dadurch gekennzeichnet, dass** der Sammler (7) mindestens im Eintrittsabschnitt der Fasern und des Restgases eine Neigung aufweist, um eine Entleerung beider zu erleichtern.

6. Ofen zur Herstellung von Kohlenstoff-Fasern nach Anspruch 1, **dadurch gekennzeichnet, dass** der Sammler (7) als geschlossener Ring ausgebildet ist, der ein Gas-Flügelrad (8) aufweist, das zur Erzeugung von zum Mitführen der erzeugten Fasern ausreichenden Gasgeschwindigkeiten geeignet ist.

7. Ofen zur Herstellung von Kohlenstoff-Fasern nach Anspruch 6, **dadurch gekennzeichnet, dass** der Ringsammler (7) durch einen Fasersammler (9) unterbrochen wird, der den Durchtritt des umlaufenden Gases nicht blockiert.

8. Ofen zur Herstellung von Kohlenstoff-Fasern nach Anspruch 6, **dadurch gekennzeichnet, dass** die gesamte Einrichtung gasdicht ist.

9. Ofen zur Herstellung von Kohlenstoff-Fasern nach Anspruch 1, **dadurch gekennzeichnet, dass** eine Rückführleitung (13) vorhanden ist, welche das Gas vom Gasumlaufsammler (7) zur Einspeisung zurückführt.

10. Ofen zur Herstellung von Kohlenstoff-Fasern nach Anspruch 9, **dadurch gekennzeichnet, dass** in der Rückführleitung (13) Steuereinrichtungen (32) für den Druck des zurückgeführten Gases vorhanden sind, um diesen innerhalb eines Bereichs an den Speisedruck anzupassen.

11. Ofen zur Herstellung von Kohlenstoff-Fasern nach Anspruch 1, **dadurch gekennzeichnet, dass** dieser alternative Speise- und/oder Entleerungsleitungen im Unterteil jedes der Reaktorrohre (1, 2, 3, 4) aufweist, die zu einem Aschesammler (28) zur individuellen Reinigung jedes Reaktorrohrs (1, 2, 3, 4) führen.

12. Ofen zur Herstellung von Kohlenstoff-Fasern nach Anspruch 11, **dadurch gekennzeichnet, dass** die alternative Einspeisung zur Reinigung aus zwei Rohrleitungen besteht, eine für Luft (24) und eine für Inertgas (23), wobei jede von diesen ein vor dem Einlass in das Reaktorrohr (1, 2, 3, 4) angeordnetes Ventil (22, 21) aufweist.

13. Ofen zur Herstellung von Kohlenstoff-Fasern nach Anspruch 12, **dadurch gekennzeichnet, dass** das Inertgas Stickstoff ist.

14. Ofen zur Herstellung von Kohlenstoff-Fasern nach Anspruch 12, **dadurch gekennzeichnet, dass** das Inertgas ein Edelgas ist.

15. Ofen zur Herstellung von Kohlenstoff-Fasern nach Anspruch 11, **dadurch gekennzeichnet, dass** die Mittel zur Entleerung während der Reinigungsoperationen aus in einer einzigen Rohrleitung zusammenlaufenden Rohren (25) bestehen, in denen am Ausgang eines jeden Reaktorrohrs (1, 2, 3, 4) ein Ventil (26) angeordnet ist.

16. Ofen zur Herstellung von Kohlenstoff-Fasern nach Anspruch 11, **dadurch gekennzeichnet, dass** der Reinigungsauslass (27) eine Steuereinrichtung (29) zur Bestimmung des Zeitpunkts aufweist, in dem der Reinigungsvorgang beendet ist.

17. Verfahren zur Herstellung von Kohlenstoff-Fasern unter Verwendung eines Ofens nach den vorhergehenden Ansprüchen, das einen kontinuierlichen Prozess zur Faserherstellung mittels Pyrolyse von Kohlenwasserstoff und Faserwachstum in der Dampfphase mit metallischen Katalysatorpartikeln in allen oder in einem Teil der Reaktionsrohre (1, 2, 3, 4) mit einer Kohlenwasserstoff-Zuführung umfasst, **dadurch gekennzeichnet, dass** weiterhin ein Katalysator (10), ein Verdünner (12) und rückgeführtes Gas (13) durch eine Steuereinrichtung bestimmten Anteilen zugeführt werden, die mit Hilfe von Massenflussreglern unabhängig auf jedes der Reaktorohre (1, 2, 3, 4) wirkt, wobei für jedes beliebige Rohr (1, 2, 3, 4) ein Reinigungsvorgang in Abhängigkeit vom Grad der Faseransammlung im Inneren eingeschaltet wird, ohne dass dieser Vorgang die Produktion in den verbleibenden Rohren (1, 2, 3, 4) beeinflusst, wobei nach Abschluss des Reinigungsvorgang eines bestimmten Rohrs in diesem anschließend die Produktionsbedingungen zur Fasersammlung in einem Mittel (9) zur Sammlung und Speicherung der Fasern wiederhergestellt werden.

18. Verfahren zur Herstellung von Kohlenstoff-Fasern nach Anspruch 17, **dadurch gekennzeichnet, dass** sich während der Herstellung von Kohlenstoff-Fasern Reaktionsrohre (1, 2, 3, 4) in Produktion und andere gleichzeitig in Reinigung befinden, ohne dass der Gesamt-Produktionsprozess durch die Reinigungsoperation gestoppt wird.

19. Verfahren zur Herstellung von Kohlenstoff-Fasern nach Anspruch 18, **dadurch gekennzeichnet, dass** die Reinigung eines Reaktionsrohrs (1, 2, 3, 4) folgende Schritte umfasst:
• Schließen der Speiseventile (19, 20) und des Entleerungsventils (6) zur Abtrennung des Rohrs von der übrigen Anlage,
• Öffnen des Inertgas-Speiseventils (21) zur Unterbrechung der Reaktion zur Bildung von Kohlenstoff-Fasern und des Ventils (26) zur Gas- und Asche-Entleerungsleitung (25),
• Aufrechterhaltung der Zufuhr von Inertgas, bis eine Steuereinrichtung (29) die Abwesenheit con Kohlenwasserstoffverbindungen feststellt,
• Schließen des Inertgas-Speiseventils (21),
• Öffnen des Luftzufuhrventils (22) zur Verbrennung der Kohlenstoff-Fasern mit Sauerstoff unter Hochtemperaturbedingungen,
• Fortsetzen der Luftzufuhr bis eine Steuereinrichtung (29) das Erlöschen der Verbrennungsreaktion bestätigt, vorzugsweise durch Feststellen des Vorhandenseins von Kohlenstoff- und Sauerstoffverbindungen,
• Schließen des Lufteinlassventils (22) und Öffnen des Inertgas-Einlassventils (21) nach Abschluss der Verbrennungsreaktion bis zur vollständigen, mittels der Steuereinrichtung (29) durch die Abwesenheit von Kohlenstoff- und Sauerstoffverbindungen festgestellten Eliminierung von Sauerstoff,
• Schließen des Inertgas-Speiseventils (21) und des Ventils (26) der Gas- und Ascheentleerungsleitung,
• erneutes Öffnen der Speiseventile (19, 20) und des Faserauslassventils (6), damit wird die Produktion in diesem Rohr wieder aufgenommen.

## Revendications

1. Four pour la fabrication de fibres de carbone, **caractérisé en ce qu'**il consiste en une série de tubes céramiques positionnés verticalement (1, 2, 3, 4), avec un bloc commun de résistances recouvertes d'un élément isolant formant un seul bloc (5), où les extrémités supérieure et inférieure des tubes (1, 2, 3, 4) sont connectées à des tubes métalliques avec des chemises de refroidissement (30) ; les tubes (1, 2, 3, 4) sont alimentés à partir des tuyaux traversants (18, 33) en amont ajustés avec des soupapes de dérivation (19, 20) ; et chacune d'eux ayant à son extrémité inférieure, après le passage de la fibre à travers le tube de réaction (1, 2, 3, 4), une soupape de dérivation (6) connectée à une extrémité à chacun des tubes métalliques correspondant à chaque tube (1, 2, 3, 4), et à l'autre extrémité à un seul collecteur (7).

2. Four pour la fabrication de fibres de carbone selon la revendication 1, **caractérisé en ce que** le bloc commun de résistances est constitué comme un regroupement de résistances individuelles associées à chaque tube de réaction (1,2,3,4).

3. Four pour la fabrication de fibres de carbone selon la revendication 1, **caractérisé en ce qu'**il a des chemises (30) qui entourent les extrémités supérieure et inférieure des tubes de réactions (1, 2, 3, 4) à travers lesquels circule le liquide de refroidissement pour la réduction de la température dans de telles extrémités en dessous de la température de pyrolyse.

4. Four pour la fabrication de fibres de carbone selon la revendication 1, **caractérisé en ce que** l'alimentation d'hydrocarbure (11), diluant (12), gaz recyclés (13), est réalisée par la répartition des quantités au moyen de contrôleurs de débit de masse (14, 15, 16, 17).

5. Four pour la fabrication de fibres de carbone selon la revendication 1, **caractérisé en ce que** le collecteur (7), au moins dans la section de réception de fibre et de gaz résiduel, a une inclination pour faciliter leur évacuation.

6. Four pour la fabrication de fibres de carbone selon la revendication 1, **caractérisé en ce que** le collecteur (7) est formé comme un anneau fermé avec un impulseur de gaz (8) avec une capacité pour générer des vitesses de gaz suffisantes pour réaliser l'extraction de la fibre produite.

7. Four pour la fabrication de fibres de carbone selon la revendication 6, **caractérisé en ce que** le collecteur d'anneau (7) est interrompu par un dispositif de collecte de fibre (9) qui ne verrouille pas le passage du gaz de recirculation.

8. Four pour la fabrication de fibres de carbone selon la revendication 6, **caractérisé en ce que** toute l'installation es étanche aux gaz.

9. Four pour la fabrication de fibres de carbone selon la revendication 1, **caractérisé en ce qu'**il existe un tuyau d'alimentation par l'arrière (13) qui conduit le gaz depuis le collecteur (7) de recirculation de gaz résiduel jusqu'à l'alimentation.

10. Four pour la fabrication de fibres de carbone selon la revendication 9, **caractérisé en ce que** dans le tuyau d'alimentation par l'arrière (13) il existe des moyens pour contrôler (32) la pression du gaz de recirculation, pour l'ajuster, dans un intervalle, à la pression d'alimentation.

11. Four pour la fabrication de fibres de carbone selon la revendication 1, **caractérisé en ce qu'**il a une alimentation alternative et des tuyaux d'évacuation dans la partie inférieure de chacun des tubes (1, 2, 3, 4), des réacteurs qui conduisent à un système de collecte de cendres (28) pour le nettoyage individualisé de chaque tube de réacteur (1, 2, 3, 4).

12. Four pour la fabrication de fibres de carbone selon la revendication 11, **caractérisé en ce que** l'alimentation alternative de nettoyage consiste en deux tuyaux, un d'air (24) et l'autre d'un gaz inerte (23), chacun d'eux avec sa soupape (22, 21) placée avant l'entrée au tube de réacteur (1, 2, 3, 4).

13. Four pour la fabrication de fibres de carbone selon la revendication 12, **caractérisé en ce que** le gaz inerte est de l'azote.

14. Four pour la fabrication de fibres de carbone selon la revendication 12, **caractérisé en ce que** le gaz inerte est un gaz noble.

15. Four pour la fabrication de fibres de carbone selon la revendication 11, **caractérisé en ce que** les moyens pour l'évacuation dans les opérations de nettoyage consistent en des tuyaux (25) qui convergent dans un seul et chacun d'eux a sa soupape (26) placée à la sortie de chaque tuyau réacteur (1, 2, 3, 4).

16. Four pour la fabrication de fibres de carbone selon la revendication 11, **caractérisé en ce que** la sortie de nettoyage (27) a un système de contrôle (29) pour déterminer le moment où a terminé l'opération de nettoyage.

17. Procédé pour l'obtention de fibre de carbone en utilisant un four selon les revendications précédentes qui consiste en un processus d'obtention de fibre par pyrolyse de l'hydrocarbure et la croissance de fibre dans la phase vapeur des particules catalytiques métalliques, dans tous ou une partie des tubes de réaction (1, 2, 3, 4) avec une alimentation en hydrocarbure (11), **caractérisé en ce qu'**il est également alimenté par un catalyseur (10), et un diluant (12) plus des gaz recyclés (13) dans des proportions déterminées par un système de contrôle qui au moyen de contrôleurs de débit de masse agit indépendamment sur chacun des tubes réacteurs (1, 2, 3, 4) ; une étape de nettoyage étant appliquée sur l'un quelconque des tubes (1, 2, 3,4), selon le degré d'accumulation de fibre à l'intérieur, sans que cette étape n'interfère dans la production du reste des tubes (1, 2, 3, 4) ; et dès que l'étape de nettoyage est appliquée à un tube donné, pour lui rendre les conditions de productions, la collecte de la fibre étant établie dans un moyen (9) de collecte et stockage.

18. Procédé pour l'obtention de fibre de carbone selon la revendication 17 **caractérisé en ce que** pendant la production de fibre de carbone, il y a des tubes de réaction (1, 2, 3, 4) dans la production et d'autres simultanément dans le nettoyage sans que le processus de production global ne soit arrêté par l'opération de nettoyage.

19. Procédé pour l'obtention de fibre de carbone selon la revendication 18, **caractérisé en ce que** le nettoyage d'un tube de réaction (1, 2, 3, 4) consiste en les étapes suivantes :
- fermeture des soupapes d'alimentation (19, 20) et de la soupape d'évacuation (6) isolant le tube du reste de l'installation.
- ouverture de la soupape d'alimentation de gaz inerte (21) pour l'arrêt de la réaction de la formation de fibre de carbone, et de la soupape (26) d'accès au tuyau d'évacuation de gaz et de cendres (25).
- maintenance de l'alimentation de gaz inerte jusqu'à ce qu'un système de contrôle (26) détecte l'absence de composés hydrocarbonés,
- fermeture de la soupape d'alimentation de gaz inerte (21),
- ouverture de la soupape d'alimentation d'air (22) pour la combustion de la fibre de carbone avec de l'oxygène dans des conditions de température élevée,
- continuation de l'alimentation d'air jusqu'à ce qu'un système de contrôle (29) confirme l'extinction de la réaction de combustion, de préférence en détectant la présence de composé de carbone et d'oxygène,
- dès que la réaction de combustion est finie, la soupape d'entrée d'air (22) est fermée et la soupape d'entrée de gaz inerte (21) est ouverte jusqu'à ce que l'oxygène soit complètement éliminé, cela étant détecté par le système de contrôle (29) grâce à l'absence de composé de carbone et d'oxygène,
- les soupapes d'alimentation de gaz inerte (21) et la soupape de tuyau d'évacuation de gaz et de cendres (26) sont fermées,
- les soupapes d'alimentation (19, 20) et les soupapes de sortie de gaz et de fibre (6) s'ouvrent à nouveau, la production étant à nouveau établie dans ce tube.
